

[54] **LOW CREEP HIGH STRENGTH FERROUS ALLOY**

[75] Inventor: **Ray H. English**, McCandless Township, Allegheny County, Pa.

[73] Assignee: **Blair-Knox Company**, Pittsburgh, Pa.

[22] Filed: **Feb. 12, 1970**

[21] Appl. No.: **11,001**

[52] **U.S. Cl.** ..... 75/128 W, 75/128 A, 75/128 P

[51] **Int. Cl.** ..... C22c 39/20

[58] **Field of Search** ..... 75/128 A, 128 W, 128 P

[56] **References Cited**

UNITED STATES PATENTS

|           |         |         |       |          |
|-----------|---------|---------|-------|----------|
| 2,557,862 | 6/1951  | Clarke  | ..... | 75/128 P |
| 2,677,610 | 5/1954  | Evans   | ..... | 75/128 P |
| 2,686,116 | 8/1954  | Schempp | ..... | 75/128 P |
| 2,984,563 | 5/1961  | Tanczyn | ..... | 75/128 W |
| 3,115,406 | 12/1963 | Balass  | ..... | 75/128 W |

|           |        |         |       |          |
|-----------|--------|---------|-------|----------|
| 3,165,400 | 1/1965 | Roy     | ..... | 75/128 A |
| 3,260,594 | 7/1966 | Ornitz  | ..... | 75/128 A |
| 3,376,780 | 4/1968 | Tanczyn | ..... | 75/128 P |
| 3,563,729 | 2/1971 | Kovach  | ..... | 75/128 P |

*Primary Examiner*—Hyland Bizot  
*Attorney, Agent, or Firm*—Buell, Blenko and Ziesenhein

[57] **ABSTRACT**

A new alloy is provided having low creep and high strength at elevated temperatures which is resistant to corrosion and thermal shock and has unusual stress rupture characteristics at elevated temperatures comprising about 0.3% to 0.9% carbon, about 20% to 30% chromium, about 15% to 35% nickel, about 0.8% to 4% manganese, about 0.9% to 3.5% silicon, about 0.3% to 5% tungsten, about 0.03% to 0.15% sulfur and the balance iron with residual impurities in ordinary amounts.

**3 Claims, No Drawings**

## LOW CREEP HIGH STRENGTH FERROUS ALLOY

This invention relates to high temperature alloys and particularly to an alloy and parts made therefrom having high strength and low creep in the temperature range 1,600° to 2,200°F. coupled with resistance to corrosion and thermal shock. The need for alloys having high strength and low creep, coupled with resistance to corrosion and thermal shock in the temperature range of 2,000°F., has long been recognized. Conventional alloys used for applications in this temperature range have not been satisfactory for most uses because of the high rate of creep, corrosion and lack of strength at temperatures at or about 1,600° to 2,200°F.

I have discovered an alloy composition having high strength and low creep characteristics coupled with corrosion resistance and high resistance to thermal shock at temperatures of about 1,600° to 2,200°F. The surprising characteristics of this alloy appear to be particularly dependent upon the control of carbon, manganese, tungsten and sulfur within a critical nickel-chromium iron base analysis. The broad composition range of the alloy of this invention lies within the following limits:

|           |                                                   |
|-----------|---------------------------------------------------|
| Sulfur    | about 0.030 to about 0.15%                        |
| Carbon    | about 0.3% to about 0.9%                          |
| Chromium  | about 17% to about 30%                            |
| Nickel    | about 15% to about 35%                            |
| Manganese | about 0.8% to about 4%                            |
| Silicon   | about 0.9% to about 3.5%                          |
| Tungsten  | about 0.3% to about 5%                            |
| Balance   | iron with residual impurities in ordinary amounts |

While the foregoing broad alloy composition will give generally satisfactory results at or above 1,800°F., I have found that for continued service above about 2,100°F. the following narrower range of composition should be observed:

|           |                                                   |
|-----------|---------------------------------------------------|
| Sulfur    | about 0.035 to about 0.100%                       |
| Carbon    | about 0.35% to about 0.75%                        |
| Chromium  | about 20% to about 30%                            |
| Nickel    | about 30% to about 35%                            |
| Manganese | about 1.2% to about 2.4%                          |
| Silicon   | about 1.2% to about 2.5%                          |
| Tungsten  | about 1.75% to about 5%                           |
| Balance   | iron with residual impurities in ordinary amounts |

A single preferred composition would be:

|           |                                                   |
|-----------|---------------------------------------------------|
| Sulfur    | about 0.075%                                      |
| Carbon    | about 0.4%                                        |
| Chromium  | about 23%                                         |
| Nickel    | about 30%                                         |
| Manganese | about 1.5%                                        |
| Silicon   | about 2%                                          |
| Tungsten  | about 1.75%                                       |
| Balance   | iron with residual impurities in ordinary amounts |

This invention is surprising in that the high sulfur in the present alloy composition appears to act precisely contrary to what would be expected. It has long been recognized that the presence of sulfur above about 0.025% in steels or iron based alloys would cause "red shortness" and the strength and resistance to cracking at high temperatures, particularly when worked or loaded, was drastically reduced. In the present alloy, on

the contrary, the presence of sulfur markedly increases the high temperature life under stress. My tests have shown that the presence of sulfur in the range here claimed will increase the stress rupture life about 4 to 9 times as compared with the same alloy having sulfur in the conventionally accepted range of 0 to 0.025%. This is a most surprising result.

The invention can perhaps be best illustrated by the following example.

### EXAMPLE

Two alloys were melted having the following compositions:

| Alloy    | C    | Mn   | Si   | Ni                    | Cr   | W    | S     |
|----------|------|------|------|-----------------------|------|------|-------|
| I        | 0.42 | 1.46 | 1.85 | 25.6                  | 22.7 | 1.42 | 0.015 |
| II       | 0.41 | 1.45 | 1.87 | 25.5                  | 22.5 | 1.44 | 0.076 |
|          |      | Bal  |      |                       |      |      |       |
| Alloy I  |      |      |      | Fe + usual impurities |      |      |       |
| Alloy II |      |      |      | Fe + usual impurities |      |      |       |

Alloy I is a recognized high temperature alloy having extraordinary stress rupture characteristics as compared with most alloys. It is sold by Blaw-Knox Company under the trade mark Mo Re No. 1 for high temperature and high stress application.

Alloy II is a composition according to the present invention.

These two alloys were formed into identical test pieces and subjected to stress rupture tests at 1,900°F. and 3,400 lbs. of stress under identical conditions.

The test piece formed from Alloy No. 1 developed 100 hours of life.

The test piece formed from Alloy No. 2 developed 883 hours of life, or almost 9 times the life of the best alloy heretofore available for high temperature high stress applications. This is a very surprising result.

The reason for this surprising result is not known to me. I believe, however, that it is the result of a redistribution of carbides in the matrix due to the presence of the sulfur in this particular alloy composition. It may, of course, be the result of the formation of a complex sulfur metal carbide composition. Whatever the mechanism, it is most unique and surprising result.

While I have described certain preferred embodiments of my invention in the foregoing specification, it will be understood that the invention may be otherwise embodied with the scope of the following claims.

I claim:

1. A low creep, high strength alloy resistant to corrosion and thermal shock at elevated temperatures and having unusual stress rupture characteristics at elevated temperatures consisting essentially of about 0.3% to 0.9% carbon, about 20% to 30% chromium, about 15% to 35% nickel, about 0.8% to 4% manganese, about 0.9% to 3.5% silicon, about 0.3% to 5% tungsten, about 0.030% to about 0.15% sulfur and the balance iron with residual impurities in ordinary amounts.

2. A low creep, high strength alloy resistant to corrosion and thermal shock at elevated temperatures having unusual stress rupture characteristics at elevated temperatures consisting essentially of about 0.35% to 0.75% carbon, about 20% to 30% chromium, about 30% to 35% nickel, about 1.2% to 2.4% manganese, about 1.2% to 2.5% silicon, about 1.75% to 5% tungsten, about 0.035% to 0.10% sulfur and the balance iron with residual impurities in ordinary amounts.

3. A low creep, high strength alloy resistant to corrosion and thermal shock at temperatures of 1,600° to 2,200° F. consisting essentially of about 0.4% carbon, about 23% chromium, about 30% nickel, about 1.5%

manganese, about 2% silicon, about 1.75% tungsten, about 0.075% sulfur and the balance iron with residual impurities in ordinary amounts.

\* \* \* \* \*

UNITED STATES PATENT OFFICE  
CERTIFICATE OF CORRECTION

Patent No. 3,856,516 Dated December 24, 1974

Inventor(s) Ray H. English

It is certified that error appears in the above-identified patent and that said Letters Patent are hereby corrected as shown below:

The name of the Assignee should read:

"BLAW-KNOX COMPANY"

Column 2, line 65, "1.75%" should read --1.75%--.

Signed and sealed this 4th day of March 1975.

(SEAL)

Attest:

RUTH C. MASON  
Attesting Officer

C. MARSHALL DANN  
Commissioner of Patents  
and Trademarks